

1

2,827,375

## POLYAMINES AS SHORT STOP AGENTS FOR AZINE COLOR DEVELOPERS

Peter Andreyev, Binghamton, N. Y., assignor to General Aniline & Film Corporation, New York, N. Y., a corporation of Delaware

No Drawing. Application March 26, 1954  
Serial No. 419,095

8 Claims. (Cl. 96—55)

The present invention relates to an improvement in the processing of light sensitive photographic materials to azine dye images, and more particularly to the use of a short stop bath which is capable of effectively removing residual azine developer from said photographic materials.

The processing of light sensitive photographic materials to azine dye images is described in U. S. P. 2,486,440, granted to W. A. Schmidt and V. Tulagin on November 1, 1949, and U. S. P. 2,570,116, granted to R. C. Gunther on October 2, 1951. These patentees recommend, as azine developers, 2,4-diamino anilines, and particularly metanilic acid derivatives, i. e., compounds containing a sulfo group meta- to one of the substituted amino groups of the 2,4-diamino anilines. Such developers to date have been found to be the most effective in producing the azine dyes. They have, however, a relatively large molecule and for this reason diffuse slowly from photographic emulsions. Furthermore, due to the presence of the sulfonic acid group, the developer and its degradation products tend to be substantive to gelatin. Because of these factors the removal of the developer from the emulsions, either as such or in the form of its degradation products, is difficult to accomplish. Thus, water washing to remove residual developer is highly impractical because of the time consumption involved.

It is recognized, however, that the residual developer must be removed prior to further chemical treatment, such as bleaching, fixing and the like, since otherwise color development fog would ensue as a consequence of the random oxidation of the residual developer by air or the silver oxidant in the bleaching bath. It was therefore suggested, the art realizing that water washing would not suffice, that short stop baths comprising a pyruvic acid (U. S. P. 2,618,559) or an acid solution of formaldehyde be employed. These solutions are satisfactory for the processing of light sensitive material on a transparent base where a certain amount of stain may be tolerated. However, it was discovered that azine images on white opaque base showed too much stain in the white or high light areas of the image to be acceptable. Neither the pyruvic acid, nor the acid formaldehyde short stop previously proposed, was sufficiently active to prevent the formation of this stain. A serious obstacle was thus presented, the application of the azine process to latent image development on the one hand, and to white opaque base material on the other hand. The realization of this obstacle has led to strenuous efforts to find more effective short stop baths than those previously described.

It has now been discovered, and rather surprisingly so, that the aforesaid stain and color development fog can be completely avoided by subjecting the light sensitive photographic material, after color development and prior to further chemical processing, to the action of a short stop bath comprising an aqueous solution of a polyamine, such as hexamethylenetetramine or its analogue glycosine.

Such short stop baths and their use in the processing of light sensitive photographic materials to azine dye images constitute the purposes and objects of my invention.

2

My short stop baths are aqueous solutions containing the polyamine in a concentration of about 1-5%. Preferably, the solutions are on the acid side and it has been found that those are most effective which have a pH from 5 to 3. It is, therefore, recommended that the baths be compounded with a non-oxidizing inorganic or organic acid, such as hydrochloric, sulfuric, phosphoric, citric, acetic, boric or the like in a concentration designed to give a pH below 7. It is to be pointed out, however, that 10 the short stop baths hereof are also effective in pH ranges as high as 8, and I, therefore, do not desire to limit myself to the use only of acid aqueous solutions of the polyamines.

I have ascertained that the short stop baths are more active when they contain, in addition to the polyamine and acid, a quantity of a clarifying agent, such as glyoxal bisulfite, and use of this reagent, although not essential, leads to better results.

The short stop baths contemplated herein are best compounded as follows:

Polyamine----- 10-50 parts by weight  
Acid----- sufficient to give pH under 7  
Water to make----- 1000 parts by weight

If a clarifying agent be used, it should be present in an amount of from 30 to 50 parts by weight.

The photographic developers utilized in producing the azine dye images are, as previously stated, those described in the aforementioned U. S. Patents 2,486,440 and 2,570,116, and particularly the metanilic acid derivatives described in these patents. Examples of such developers are 4-( $\beta$ -hydroxyethylamino)-6-phenylamino-metanilic acid; 4 - ( $\beta$  - hydroxyethylamino) - 6 - methylamino - metanilic acid; 4 - ( $\beta$  - hydroxy -  $\beta$  - methyl - ethyl amino)-6-phenylamino-metanilic acid and the like.

The azine dyes resulting from the use of such developers are formed through the action of the oxidation products of the developers on color formers of the type described in the aforesaid patents. Preferably, the color formers are located in the emulsion layers and, to this end, they contain a group which renders them non-migratory in the emulsion layers. For practical purposes it is recommended that the photographic material containing the color formers be in the form of an integral tripack.

The processing of the light sensitive photographic material is substantially the same as described in U. S. P. 2,618,559, excepting that the pyruvic acid short stop solution of the patent is replaced by a short stop bath as described herein. It is to be pointed out that rinsing with oxygenated water following color development and preceding the short stop treatment tends to produce color development fog. It is, therefore, preferable to interpolate the short stop between the color development and bleaching steps. It is possible, however, to incorporate after color development and prior to short stopping a rinse treatment with a strong aqueous solution of sodium bisulfite. This adds an extra step to the processing, however, and hence should be used only where circumstances demand its employment.

The following examples will serve to further illustrate the invention, the parts being by weight unless otherwise stated.

## Example I

An integral tripack with a bottom layer composed of a red sensitive emulsion containing phenyl-J-acid-N-octadecyl urethane; a middle layer composed of a green sensitive emulsion containing 2-stearoylamine-6-(8-hydroxy-cinchoninoylamino)-toluene-4-sulfonic acid, and a top layer composed of a blue sensitive emulsion containing 2 - (4 - benzoylacetaminophenyl) - 1-octadecyl-5-benzimi-

dazole sulfonic acid was exposed and the latent image developed in a developer of the following composition:

|                                                              | Grams |
|--------------------------------------------------------------|-------|
| Sodium carbonate, monohydrate                                | 40    |
| Sodium sulfite                                               | 60    |
| Potassium bromide                                            | 5     |
| Pyridine                                                     | 16    |
| Benzylamine                                                  | 1     |
| 4-( $\beta$ -hydroxyethylamino)-6-phenylamino-metanilic acid | 5     |
| Water to make 1000 cc.                                       |       |

After color development, the film was rinsed and treated for 5 minutes in a bath of the following composition:

|                        | Grams |
|------------------------|-------|
| Glyoxal bisulfite      | 40    |
| Hexamethylenetetramine | 40    |
| Citric acid            | 128   |
| Water to make 1000 cc. |       |

The film was washed, bleached in a ferricyanide bleach and fixed in an acid hardening solution. There were thus obtained multicolor stain and fog free negative dye images.

#### Example II

Three color separation negatives were printed onto a film having a white opaque base, but otherwise constituted as in Example VI of U. S. P. 2,570,116. The film was then developed in a latent image developer compounded as follows:

| (A)                            |       |       |
|--------------------------------|-------|-------|
| Water                          | cc.   | 800   |
| 2-aminopyridine sulfate        | grams | 3.1   |
| Sodium tetra acetic acid       | do    | 1.0   |
| Sodium sulfite (anhydrous)     | do    | 15.0  |
| Sodium carbonate (monohydrate) | do    | 60.0  |
| Sodium bromide                 | do    | 0.86  |
| Sodium sulfate                 | do    | 100.0 |
| Trisodium phosphate            | do    | 13.5  |
| Sodium bisulfite               | do    | 1.0   |
| Water to make 900 cc.          |       |       |

| (B)                                                          |       |     |
|--------------------------------------------------------------|-------|-----|
| Water                                                        | cc.   | 100 |
| Sodium sulfite                                               | grams | 5.0 |
| 4-( $\beta$ -hydroxyethylamino)-6-phenylamino metanilic acid | grams | 5.8 |
| Add B to A just before using.                                |       |     |

Immediately after color development, the film was subjected to the action of a short stop bath having the following constitution:

|                                            |       |      |
|--------------------------------------------|-------|------|
| Hexamethylenetetramine                     | grams | 25   |
| Hydrochloric acid sufficient to give pH 2. |       |      |
| Water                                      | cc.   | 1000 |

The film was then bleached in a ferricyanide bleach and fixed in an acid hardening hypo. The dye images obtained were completely free from stain and color development fog.

#### Example III

The procedure is the same as in Example II, excepting that the hexamethylenetetramine was replaced by an

equivalent amount of glycosine added to the short stop bath.

Various modifications of the invention will occur to those skilled in the art and I, therefore, do not intend to be limited in the patent granted except as necessitated by the appended claims.

I claim:

1. A photographic stop bath effective to remove residual azine developer from light sensitive photographic emulsions comprising an aqueous solution of a polyamine selected from the class consisting of hexamethylenetetramine and glycosine, said solution including glyoxal bisulfite as a clarifying agent, and containing sufficient acid to produce a pH below 7.

5 2. The stop bath as defined in claim 1, wherein the polyamine is present in a concentration of 1-5% by weight of the solution.

10 3. A photographic stop bath effective to remove residual developer from light sensitive photographic emulsions comprising an aqueous solution of 10-50 parts by weight of a polyamine selected from the class consisting of hexamethylenetetramine and glycosine, glyoxal bisulfite as a clarifying agent, and sufficient acid to provide a pH of from 2 to 3.

15 4. The composition as defined in claim 3, wherein the polyamine is hexamethylenetetramine.

20 5. In the process of producing subtractively colored azine dye images in a silver halide emulsion layer containing a color former capable of coupling with the oxidation products of 2,4-diamino aniline developing agent to form an azine dye which comprises exposing the emulsion and developing the same with a color developer containing a 2,4-diamino aniline as the effective developing agent, the improvement which comprises avoiding the formation of color development fog and stain after color development and prior to bleaching by short stopping the color developed emulsion with an aqueous solution of a polyamine selected from the class consisting of hexamethylenetetramine and glycosine and containing sufficient acid to produce a pH below 7.

25 6. The process as defined in claim 5, wherein the short stop bath contains the polyamine in a concentration of 1-5% by weight.

30 7. The process as defined in claim 5, wherein the short stop bath contains glyoxal bisulfite as a clarifying agent.

35 8. The process as defined in claim 5, wherein the short stop bath contains per liter of water 40 grams of glyoxal bisulfite, 40 grams of hexamethylenetetramine and sufficient acid to give a pH of from 2 to 3.

#### References Cited in the file of this patent

#### UNITED STATES PATENTS

|           |         |               |
|-----------|---------|---------------|
| 2,618,559 | Gunther | Nov. 18, 1952 |
| 2,657,139 | Bates   | Oct. 27, 1953 |

#### FOREIGN PATENTS

|         |               |              |
|---------|---------------|--------------|
| 294,972 | Great Britain | Aug. 3, 1928 |
|---------|---------------|--------------|

#### OTHER REFERENCES

|                                                                              |  |
|------------------------------------------------------------------------------|--|
| Chemical Abstract, 29, 4655 (Note 9), 1935.                                  |  |
| Merck Index, publ. by Merck & Co., Rahway, N. J., fifth ed., 1940, page 353. |  |